

## UNITED STATES PATENT OFFICE

2,388,826

## YARN CONDITIONING PROCESS

John E. Caldwell, Kingsport, Tenn., assignor to  
 Eastman Kodak Company, Rochester, N. Y., a  
 corporation of New Jersey

No Drawing. Application February 22, 1944,  
 Serial No. 523,477

4 Claims. (Cl. 117—139.5)

This invention relates to the conditioning of textile yarns, and particularly to the conditioning of yarns, threads, filaments and fibers composed of or containing organic derivatives of cellulose such as cellulose acetate, cellulose propionate, cellulose butyrate, cellulose acetate propionate and cellulose acetate butyrate, to render such materials amenable to various textile operations such as knitting, weaving, carding, spinning, twisting and the like.

As is well known in the textile industry, the manufacture, processing and use of yarns composed of or containing organic derivatives of cellulose and similar synthetic materials give rise to numerous problems generally absent from the handling of natural yarns such as silk, wool, cotton and the like. One of the chief problems encountered in dealing with these synthetic materials is to so lubricate or soften and, in some instances, to both lubricate and soften, the yarn in question that it will have the correct frictional characteristics, or drag, and the required flexibility for the specific purpose in view. In the handling of continuous filament yarn, for example, it is necessary to condition the material to reduce the tendency toward breakage of individual filaments when the yarn is subjected to mechanical strains such as are involved in passage of the yarn over rolls, guides, and other parts of the yarn-producing mechanism and in twisting, winding, reeling and similar operations. In the case of yarns intended for use on commercial knitting machinery, it is particularly important that the yarn be soft and pliable in order that it may conform to the contour of the needles and give a closely knit fabric free from cuts, pinholes, stitch distortion, laddering, misplaits and other common defects.

Another problem of major proportions presented by these synthetic yarns is their extreme tendency to pick up charges of static electricity, especially in such operations as twisting, winding, warping, picking, carding, combing, drafting, spinning, and the like. This tendency is particularly aggravated in the case of cut staple fibers, since in the commercial use of such material it is normally subjected to a number of extremely severe operations such as picking, carding and combing, all of which tend to so charge the individual fibers as to make proper web formation difficult or impossible or to give the ultimate yarn an undesirable unevenness.

In some types of yarn, all three of the above-mentioned problems of lubrication, softening and anti-static treatment are present and in any case

the matter of providing a yarn conditioning composition, in which the several functions are properly coordinated to accomplish the desired result is often a matter of extreme difficulty. This is due to the fact that in any given yarn conditioning composition, whether primarily designed for use as a warp, filling or knitting lubricant, or as an anti-static, the various components and their functions must be delicately balanced one against

10 the other so as to give a practical and commercially satisfactory yarn treatment.

Textile yarn treating compositions are generally applied in one of two forms, that is, a clear oil or an aqueous or other emulsion thereof. If 15 the composition is to be applied in the form of an oil, it is important that it should remain a clear, homogeneous liquid and not separate into two or more phases on standing. In many instances, it is necessary to employ blending or 20 solubilizing agents in order to preclude the possibility of such separation. In the case of emulsions, on the other hand, it is often necessary to employ agents which function to cause the various components of the composition to be effectively and permanently dispersed throughout the 25 dispersing medium. In addition it is, in general, necessary in those cases where the yarn treating composition contains oils or oily materials which are normally insoluble in water to add emulsifying agents for the purpose of enabling these components to be removed from the yarns or fabrics to which they are applied in the ordinary aqueous scour baths.

The present invention has as its principal object to provide an improved process for the conditioning of textile yarns, threads, filaments and fibers, particularly those composed of or containing organic derivatives of cellulose such as cellulose acetate, cellulose propionate, cellulose butyrate, cellulose acetate propionate and cellulose acetate butyrate, to render such materials amenable to various textile operations and processes, such as knitting, weaving, spinning, carding, drawing and the like. A further object is to provide an improved process for the lubrication and improvement of hand of such yarns. A still further object is to provide improved yarn treating compositions containing one or more oils and having a high degree of stability even when kept for long periods of time. Another object is to provide an improved yarn conditioning agent or composition of the emulsion type which contains one or more oils and an emulsifying agent permitting the various components to be readily scoured from the yarns or fabrics to which they

may be applied. A specific object is to provide a yarn conditioning composition containing an agent which can function, both as a lubricant and as a blending or solubilizing agent between a mineral oil and another normally incompatible oil or a soap which is normally insoluble in mineral oil. Other objects will appear hereinafter.

These objects are accomplished by the following invention which, in its broader aspects, comprises treating yarns, threads, filaments or fibers, particularly those composed of or containing organic derivatives of cellulose, such as cellulose acetate, cellulose propionate, cellulose butyrate, cellulose acetate propionate and cellulose acetate butyrate, with stable yarn treating compositions or conditioning agents which are readily susceptible of removal from the yarn by means of ordinary aqueous scour baths, characterized by the fact that such compositions are composed of or contain high molecular weight nitriles derived from fatty acids containing 8-20 carbon atoms.

I have found that the nitriles possess unique and exceptionally valuable properties, not only as yarn lubricants per se, but as constituents of various yarn treating compositions or lubricants. While I limit myself to no theory regarding the efficacy of the nitriles as ingredients of yarn conditioning compositions, it is my belief that their exceptional lubricating properties may be attributed to the fact that they contain a long hydrocarbon chain. The presence of the long hydrocarbon chain also imparts solubility of these compounds in various hydrocarbon oils commonly employed as ingredients of yarn lubricating compositions and makes possible their use in association with said oils. In addition, these compounds are characterized by the presence of a nitrile or  $-C\equiv N$  group which imparts miscibility with polar compounds such as soaps, sulfonated oils, fatty alcohol sulfates and other compounds employed as emulsifying or dispersing agents in the compounding of textile conditioning compositions. The polar nitrile group also has the advantage that it permits high film strength and adhesion in the lubricating film deposited on the yarn.

I have by extensive experimentation demonstrated that the long chain nitriles possess a most unusual and unexpected ability to lubricate yarns to which they are applied, particularly yarns composed of or containing organic derivatives of cellulose such as cellulose acetate and similar cellulose organic acid esters and like materials. Moreover, these compounds are bi-functional in that they combine the properties of a lubricant and a blending agent in one individual compound, that is, they can function not only as lubricants per se, or in association with other lubricants, but they have the unusual property of blending or solubilizing in various hydrocarbon oils, many compounds such as soaps, sulfonated oils and the like employed as dispersing or emulsifying agents in textile conditioning compositions which are normally insoluble in, or incompatible with, such oils. In addition, since they are chemically neutral, the long-chain nitriles exert no deleterious action upon the yarn fibers themselves, nor do they induce corrosion of the metal parts of the yarn producing or processing machinery with which they may come in contact.

I have found that both the liquid and solid long-chain nitriles are of value as yarn lubricants. Those which are liquid at ordinary temperatures may be applied as such to the yarn as lubricants, while those which are solid at ordi-

nary temperatures may be dissolved in suitable inert hydrocarbon or other solvents. In either case, these compounds may be employed as constituents of multi-component yarn conditioning agents containing appropriate mineral, animal and vegetable oils, fats and waxes or other appropriate materials generally employed in the compounding of textile lubricants. As indicated above, when applied alone or in combination with other conditioning agents, such as oils or waxes, they impart to textile yarns a very low coefficient of friction between the yarn surface and the surface of steel or porcelain guides such as are commonly employed in the textile industry. When applied, either alone or in combination with other yarn conditioning agents, they impart a soft, smooth hand or feel to the yarn and greatly reduce the harshness or scroop generally resulting from the use of ordinary textile lubricants such as mineral oil.

The nitriles may be readily prepared by any of the well-known standard procedures for the preparation of this class of compounds described in the chemical literature. The best method for preparing the nitriles is through pyrolysis of the acid in the presence of ammonia as described by Ralston and Harwood, J. Am. Chem. Soc. 59, 986 (1937); U. S. Patent No. 2,061,314. The physical properties of the straight chain fatty acid nitriles are described by Ralston, Selby, and Pool, Ind. Eng. Chem. 33, 682 (1941). The high molecular weight nitriles employed in the process of the invention may be prepared by treating the corresponding carboxylic acid amide with phosgene as outlined in British Patent No. 488,036. They may also be produced by treating the carboxylic amides with thionyl chloride, as described by Oldham, J. Chem. Soc. 1939, p. 201. Polymerized fatty acid nitriles may be prepared according to the method described in British Patent No. 488,808.

Among suitable long-chain nitriles which may be employed in accordance with my invention as yarn lubricants per se or as ingredients of yarn lubricating and conditioning compositions are those derived from straight-chain saturated acids, unsaturated acids, naphthenic acids, dibasic acids and various mixed acids such as those present in naturally-occurring fats and oils such as coconut oil, olive oil and tallow. Typical examples of specific compounds are as follows:

#### *Nitriles from saturated acids*

Lauroonitrile  
Myristonitrile  
Palmitonitrile  
Margaronitrile  
Stearonitrile

#### *Nitriles from unsaturated acids*

Oleonitrile  
Elaidonitrile  
Linolenonitrile

#### *Substituted nitriles*

Ricinoleic acid nitrile  
Nitrile of 9-phenyl stearic acid  
9-hydroxy nonanenitrile  
2-phenyl acetonitrile  
3-phenyl propionitrile  
9,10-dichloro octadecanenitrile

#### *Nitriles of dibasic acids*

Suberonitrile  
Azeleonitrile  
Sebaconitrile

*Mixed nitriles*

Nitriles of coconut oil fatty acids  
Nitriles of olive oil fatty acids  
Nitriles of tallow fatty acids

In these compounds the nitrile may contain other groups or substituents, as would be the case with ricinoleic acid nitrile and the nitrile of 9-phenyl stearic acid. Additional examples of nitriles derived from saturated acids are caprylonitrile, 10 pelargononitrile, capronitrile, undecanenitrile, tridecanenitrile, pentadecanenitrile, eicosanenitrile, 15 2-ethyl hexanenitrile, 2-butyl hexanenitrile, and 3-ethyl octanenitrile. Nitriles derived from naphthenic acids containing 8-20 carbon atoms may also be employed as above described.

As indicated above, the long-chain nitriles may be used alone or in combination with other yarn conditioning agents. For example, oleonitrile may be applied to yarn in various stages of processing by means of wick, roll, spray, etc., to the extent of 0.3-10.0% based on the weight of the yarn. Nitriles which are solids or semi-solids at room temperature may be dissolved in a volatile solvent such as toluene or a suitable petroleum fraction, and applied by known means. Yarns lubricated in this way are characterized by extremely low friction when passed through porcelain or steel guides.

The nitriles have their widest application as a component of mixed oils or lubricants. Because of their molecular structure which embodies a relatively long hydrocarbon chain in combination with the polar nitrile group  $-C\equiv N$ , they are valuable blending agents. The hydrocarbon chain imparts the property of solubility in oils, while the nitrile group tends to give miscibility with polar compounds such as sulfonated oils, soaps, fatty alcohol sulfates, etc. Thus it is found that certain highly sulfonated olive and 30 castor oils will form turbid solutions when mixed with mineral oil. If a high molecular weight nitrile or mixture of such nitriles is used as a third component of the formula, a clear, homogeneous solution results.

The nitriles are excellent solvents for soaps and other emulsifying or dispersing agents. Thus, for example, oleic and stearic acid amine soaps when mixed with oleonitrile or the nitriles obtained from lard oil fatty acids form clear, stable solutions which may be applied to textile fibers by the usual methods. Alternatively, the solution of soap in the nitrile may be mixed with other oils, fats, or waxes to form conditioning agents of diverse types.

The nitriles not only lend themselves readily to the formation of stable oils, but also are easily adaptable to emulsification processes. For example, a solution of soap and/or sulfonated oil in oleonitrile or stearonitrile forms a finely dispersed, stable emulsion when mixed with water. Or the nitrile soap solution may be mixed with a mineral oil and/or a vegetable oil and the whole emulsified by suitable treatment with water.

My invention will be more fully understood by reference to the following examples which are included merely for purposes of illustration and not as a limitation thereof.

*Example 1*

Continuous filament, 150 denier, cellulose acetate warp yarn is lubricated by the application thereto of lauronitrile. In this case the nitrile is applied as such in an amount corresponding to 4%, based on the weight of the yarn by means

of an applicator roll or equivalent device. It was found that when the lubricated yarn was passed over porcelain and steel guides that the friction, as measured by the grams pull developed in the yarn was appreciably lower than that developed in similar yarn lubricated with ordinary textile lubricants.

*Example 2*

A cellulose acetate yarn similar to that of Example 1 was treated under the same conditions with 5% of stearonitrile. In this case the friction was also appreciably reduced below that developed when treating the same yarn with other textile lubricants.

*Example 3*

A cellulose acetate yarn of the same type as that referred to in Example 1 was treated by the application thereto of 3% of oleonitrile. Again 20 the friction was reduced below that obtained by the application to the same yarn of ordinary textile lubricants.

A comparison of the improved results to be obtained in the lubrication of textile yarns by means of the nitriles and by means of ordinary 25 yarn lubricants can be obtained by reference to the following table which embodies the results of tests run on the same type of cellulose acetate yarn lubricated with the same amounts of several different lubricants under identical conditions. The amount of friction or drag produced as these 30 lubricated yarns were drawn over both porcelain and steel guides was measured on a machine adapted for this purpose. The figures used in 35 the table represent the grams of force required to pull the lubricated yarn over the porcelain and steel guides.

| Lubricating agent     | Grams pull developed |              |
|-----------------------|----------------------|--------------|
|                       | Porcelain guides     | Steel guides |
| Lauronitrile          | 22                   | 14.5         |
| Stearonitrile         | 19                   | 19           |
| Oleonitrile           | 20                   | 19           |
| Soy bean oil          | 26                   | 29           |
| Olive oil             | 27                   | 29           |
| Neat's-foot oil       | 27                   | 29           |
| Lard oil              | 28                   | 30           |
| Oleic acid            | 28                   | 31           |
| Castor oil            | 34                   | 39           |
| Blown neat's-foot oil | 38                   | 39           |
| Glycol oleate         | 27                   | 41           |

The yarn employed in running the tests from which the above data were obtained was 150-denier, bright luster cellulose acetate yarn twisted to three turns per inch.

*Example 4*

A cellulose acetate yarn is lubricated by the application of a clear oil having the following composition:

|                              | Parts |
|------------------------------|-------|
| Sulfonated olive oil         | 30    |
| Mineral oil (55 secs. visc.) | 55    |
| Oleonitrile                  | 15    |

In this formula the oleonitrile functions not only as a lubricant, but also as a blending agent or co-solvent between the mineral oil and the sulfonated olive oil. A clear, homogeneous solution is formed by the combination of these various ingredients which will not separate into phases on standing. The conditioning fluid may be applied as such by means of a wick, roll or equivalent device or it may be dispersed in water and applied as an emulsion.

## Example 5

A clear, stable homogeneous 10% aqueous emulsion may be prepared by dispersing 10 parts by weight of the following formula in 90 parts of water.

|                              | Parts |
|------------------------------|-------|
| Mineral oil (55 secs. visc.) | 60    |
| Triethanolamine oleate       | 27    |
| Lauronitrile                 | 13    |

Triethanolamine oleate is insoluble in mineral oil, but a clear, homogeneous, stable solution may be prepared by employing lauronitrile as a blending agent or cosolvent in the proportions shown above. This composition may be applied to fibers in various stages of processing as an oil or as an aqueous emulsion.

## Example 6

A composition which may be employed as a clear, homogeneous stable oil, or as an aqueous emulsion, may have the following composition:

|                  | Parts |
|------------------|-------|
| Coconut oil      | 60    |
| Stearonitrile    | 40    |
| Stoddard solvent | 200   |

This composition may be applied to filaments or fibers of cellulose acetate or other cellulose organic acid esters to the extent of 0.5 to 5.0% based on the weight of the yarn. It imparts to the yarn an extremely low coefficient of friction.

The particular method of application of the yarn treating compositions of my invention to the yarn will depend largely upon the nature of the yarn and the use for which it is intended. In general, the compositions may be applied by any of the standard procedures such as roll, wick, bath, or spray application. If the yarn is in continuous filament form, compositions may be applied just as the yarn emerges from the spinning cabinet, or while passing from package to package. Likewise, the lubricant may be applied during twisting, winding, creping or similar operations. In the case of cut staple fibers, the compositions may be conveniently applied in the form of an emulsion bath or spray, preferably after any desired special treatment of the yarn such as crimping or the like.

While I have found it convenient to describe my invention with particular reference to the treatment of yarns composed of or containing organic derivatives of cellulose, particularly cellulose acetate, the conditioning agent and compositions described herein are also applicable to the conditioning of many other types of cellulose derivative yarns, such as those composed of or containing cellulose propionate, cellulose butyrate, cellulose acetate propionate, cellulose acetate butyrate, the cellulose ethers such as ethyl, methyl and benzyl celluloses, viscose and cuprammonium cellulose, silk, wool, cotton and other natural and artificial materials.

The term "yarn" as used herein and in the claims is to be understood as covering single filaments, a plurality of filaments associated in the form of roving, threads and the like, either of high or low twist, composite threads or yarns composed of a mixture of natural and artificial filaments, composite threads formed by twisting together individual threads or strands of the same or different natural or artificial materials of the same or different deniers, creped or crimped yarns, and crimped or uncrimped cut staple fibers produced from natural or artificial filaments, and spun yarn produced from such staple fibers.

As indicated above, my invention resides in the discovery that the long-chain nitriles give outstanding results as yarn lubricating agents, particularly as lubricating and conditioning agents for yarns composed of or containing cellulose acetate and similar cellulose organic acid esters, as well as the fact that they are outstanding in their ability to operate as blending agents between mineral oils and soaps, sulfonated oils and other emulsifying or dispersing agents which are normally insoluble in mineral oils. The compositions of my invention are characterized by the fact that, not only are they excellent lubricants, but they are also readily susceptible of removal from yarns or fabrics by the ordinary aqueous scour baths customarily employed in the textile industry.

Of the various nitriles referred to above, I have found that lauronitrile, stearonitrile and oleonitrile are outstanding and unique in their ability to impart low friction characteristics to cellulose acetate and other textile yarns lubricated therewith.

What I claim and desire to secure by Letters Patent of the United States is:

1. The process of conditioning a cellulose organic derivative textile yarn to render the yarn amenable to textile operations such as knitting, weaving, spinning, carding, drawing and the like, which comprises applying thereto a lubricating composition containing a compound having the graphic formula  $C_nH_{2n-1}CN$  where  $n$  is 7 to 19 carbon atoms.

2. The process of conditioning yarn composed of or containing cellulose acetate to render it amenable to knitting, weaving, spinning, carding, drawing and the like which comprises applying thereto a composition containing lauronitrile.

3. The process of conditioning yarn composed of or containing cellulose acetate to render it amenable to knitting, weaving, spinning, carding, drawing and the like which comprises applying thereto a composition containing stearonitrile.

4. The process of conditioning yarn composed of or containing cellulose acetate to render it amenable to knitting, weaving, spinning, carding, drawing and the like which comprises applying thereto a composition containing oleonitrile.

JOHN R. CALDWELL.